# EUROPEAN PATENT SPECIFICATION

(11) **EP 2 714 859 B1**
(45) Date of publication and mention of the grant of the patent: **26.12.2018**
(21) Application number: 12729033.6
(22) Date of filing: 30.05.2012
(51) Int. Cl.: C10L 1/14

(54) **LIQUID FUEL COMPOSITIONS**
FLÜSSIGE KRAFTSTOFFZUSAMMENSETZUNGEN
COMPOSITIONS DE CARBURANT LIQUIDE

(30) Priority: 30.05.2011 EP 11168052
(43) Date of publication of application: 09.04.2014
(73) Proprietor: Shell Internationale Research Maatschappij B.V., 2596 HR The Hague (NL)
(72) Inventor: BREWER, Mark Lawrence, Ince Chester CH2 4NU (GB); SMITH, Susan Jane, Ince Chester CH2 4NU (GB)
(74) Representative: Shell Legal Services IP
(86) International application number: PCT/EP2012/060085
(87) International publication number: WO 2012/163935

(56) References cited:
- EP-A1- 0 634 472
- EP-A1- 0 707 058
- EP-A1- 0 947 576
- WO-A1-02/079353
- US-A- 4 920 691
- US-A1- 2006 223 718
- CHEVRON PHILLIPS COMPANY: "Safe Handling and Storage of Synfluid Polyalphaolefins (PAO)", 20080108 , 8 January 2008 (2008-01-08), pages 1-27, XP002600842, Retrieved from the Internet: URL:http://www.cpchem.com/bl/pao/en-us/Doc uments/PAO_2008_Rev_0.pdf [retrieved on 2010-09-23]

## Description

### Field of the Invention

The present invention relates to a liquid fuel composition. The present invention also relates to a method of improving the fuel economy performance of an internal combustion engine by fuelling the internal combustion engine with the liquid fuel composition described hereinbelow.

### Background of the Invention

Government regulations and market demands continue to emphasize conservation of fossil fuels in the transportation industry. There is increasing demand for more fuel-efficient vehicles in order to meet CO₂ emissions reductions targets. Therefore, any incremental improvement in fuel economy (FE) is of great importance in the automotive sector. Lubricants can play an important role in reducing a vehicle's fuel consumption and there is a continuing need for improvements in fuel economy performance of lubricant compositions contained within an internal combustion engine.

R.I. Taylor & R.C. Coy, "Improved Fuel Efficiency by Lubricant Design: A Review", Proc Instn Mech Engrs, Vol 214, Part J, pp 1-15, 2000, reviews the properties of the lubricant composition that affect fuel consumption. In particular, this review paper teaches that one of the properties of a lubricant composition which affects the fuel economy performance of that lubricant composition is viscosity. The lower the viscosity of the lubricant composition, the greater the fuel economy performance of that lubricant composition [SAE 982502]. However, viscosity increase is often observed during an oil drain interval (ODI) [SAE 2008-01-1740], which is expected to be detrimental to fuel economy.

While the lubricant formulation remains fixed from the beginning, an opportunity has been identified to influence the lubricant positively via the fuel composition, in particular by adding certain fuel additives to the fuel composition.

Viscosity control additives such as polyalphaolefins and esters are known for use in liquid fuel compositions and have been disclosed in the following patent publications: EP-A-707058; EP-A-290088; EP-A-634472; WO98/11178 and WO98/11177.

EP-A-707058 discloses a fuel composition comprising a gasoline base fuel, a polyalphaolefin and a detergent which may be a polyisobutylenyl succinimide or an aliphatic or alkoxylated polyamine. EP-A-634472 also discloses a fuel composition comprising a gasoline base fuel, a polyalphaolefin and a succinimide. A detergent in a fuel composition aids performance by cleaning the internal parts of an engine during use and reducing engine deposits. Detergents in general, and succinimide derivatives in particular, do not contribute significantly to lubricity and reduced friction, and are not therefore known to act as friction modifiers, nor to aid fuel economy via friction reduction.

It has now surprisingly been found that the use of selected viscosity control additives having certain physical properties together with selected friction modifiers in liquid fuel compositions can provide benefits in terms of improved fuel economy and improved engine lubricant performance.

### Summary of the Invention

The present invention provides a liquid fuel composition comprising:
(a) a base fuel suitable for use in an internal combustion engine, wherein the base fuel is a gasoline fuel;
(b) a first fuel additive selected from one or more viscosity control agents having:
   (i) a kinematic viscosity at 100°C of 27 mm²/s or less; and
   (ii) a NOACK volatility at 250°C of 100 %wt, preferably 20 %wt or less; and
(c) a second fuel additive selected from one or more friction modifiers, wherein the one or more friction modifiers is selected from alkoxylated amines;
wherein the first fuel additive is PAO-2, and wherein the liquid fuel composition is a gasoline fuel composition.

The present invention further provides a method of improving the fuel economy performance of an internal combustion engine, said method comprising fuelling an internal combustion engine containing an engine lubricant with a liquid fuel composition comprising:
(a) a base fuel suitable for use in an internal combustion engine, wherein the base fuel is a gasoline fuel;
(b) a first fuel additive selected from one or more viscosity control agents having:
   (i) a kinematic viscosity at 100°C of 27 mm²/s or less; and
   (ii) a NOACK volatility at 250°C of 100 %wt, preferably 20 %wt or less; and
(c) a second fuel additive selected from one or more friction modifiers, wherein the one or more friction modifiers is selected from alkoxylated amines;
wherein the first fuel additive is PAO-2, and wherein the liquid fuel composition is a gasoline fuel composition.

### Detailed Description of the Invention

The liquid fuel composition of the present invention comprises a base fuel suitable for use in an internal combustion engine, a first fuel additive selected from viscosity control agents having certain physical properties and a second fuel additive which is a friction modifier. The base fuel suitable for use in an internal combustion engine is a gasoline fuel, and therefore the liquid fuel composition of the present invention is a gasoline fuel composition.

As used herein, the term "viscosity control additive" or "VCA" is a fuel-borne additive intended to control increases in lubricant viscosity. As used herein, the term "friction modifier" or "FM" is an additive intended to reduce the coefficient of friction, normally in the boundary lubrication regime.

The first fuel additive used in the liquid fuel composition herein is a viscosity control agent (VCA) and has a kinematic viscosity at 100°C (as measured by ASTM D 445 or IP71) of 27 cSt or less. Preferably, the kinematic viscosity at 100°C (as measured by ASTM D 445) additionally accords with one or more of the parameters listed below:
(i) 22 cSt or less;
(ii) 17 cSt or less;
(iii) 13 cSt or less;
(iv) 10 cSt or less;
(v) 8 cSt or less;
(vi) 6 cSt or less;
(vii) 5.5.cSt or less;
(viii) At least 2 cSt;
(ix) At least 3 cSt;
(x) At least 3.5 cSt;
(xi) At least 4 cSt;
(xii) At least 4.5 cSt.

In preferred embodiments herein the first fuel additive has a kinematic viscosity at 100°C (as measured by ASTM D 445) in the range of from 2 cSt to 8 cSt, preferably in the range of from 3 cSt to 8 cSt, more preferably in the range of from 3.5 cSt to 6 cSt, even more preferably in the range of from 4 cSt to 6 cSt, especially in the range of from 4 cSt to 5.5 cSt, more especially in the range of from 4.5 cSt to 5.5 cSt.

In addition, the first fuel additive used in the liquid fuel composition herein has a NOACK volatility (as measured by ASTM D5800 at 250°C) of 100 wt% or less, preferably 20 wt% or less, preferably 10 wt% or less, more preferably 6 wt% or less, even more preferably 5 wt% or less, especially 4 wt% or less.

The viscosity control agent for use as the first fuel additive herein is the polyalphaolefin PAO-2.

Poly-alpha olefin base oils (PAOs) and their manufacture are well known in the art. Preferred poly-alpha olefin base oils that may be used in the fuel compositions of the present invention may be derived from linear C₂ to C₃₂, preferably C₆ to C₁₆, alpha olefins. Particularly preferred feedstocks for said poly-alpha olefins are 1-octene, 1-decene, 1-dodecene and 1-tetradecene. Poly-alpha olefins can be prepared from single component streams or mixed component streams.

Commercially available polyalphaolefins for use herein include that available from Ineos under the tradename Durasyn 162; that available from Chevron Corporation under the tradename Synfluid PAO 2; and that commercially available from Neste under the tradename Nexbase 2002.

Preferably, the amount of the first fuel additive having a viscosity of less than 27 cSt and a NOACK volatility of 100 %wt or less, preferably 20 %wt or less, present in the liquid fuel composition of the present invention is at least 5 ppmw (parts per million by weight), based on the overall weight of the liquid fuel composition. More preferably, the amount of first fuel additive present in the liquid fuel composition of the present invention additionally accords with one or more of the parameters (i) to (xx) listed below:
(i) at least 10 ppmw
(ii) at least 20 ppmw
(iii) at least 30 ppmw
(iv) at least 40 ppmw
(v) at least 50 ppmw
(vi) at least 100 ppmw
(vii) at least 200 ppmw
(viii) at least 300 ppmw
(ix) at least 400 ppmw
(x) at least 500 ppmw
(xi) at least 600 ppmw
(xii) at least 700 ppmw
(xiii) at least 800 ppmw
(xiv) at least 900 ppmw
(xv) at least 1000 ppmw
(xvi) at least 2500ppmw
(xvii) at most 5000ppmw
(xviii) at most 10000 ppmw
(xix) at most 2 %wt.
(xx) at most 5 %wt.

It should be noted that the base fuel may already contain minor amounts of fuel additives, such as alkyl benzenes or alkyl naphthenates, and the amount of at least 10 ppmw, and each of the amounts listed in (i)-(xx) above is in addition to any minor amounts of such fuel additives which may already be present in the base fuel.

The liquid fuel compositions of the present invention further comprise, as an essential component, a second fuel additive which is selected from one or more friction modifiers wherein the one or more friction modifier is selected from alkoxylated amines.

Preferably, the amount of the second fuel additive in the liquid fuel composition of the present invention is at least 10 ppmw (parts per million by weight), based on the overall weight of the liquid fuel composition. More preferably, the amount of second fuel additive present in the liquid fuel composition of the present invention additionally accords with one or more of the parameters (i) to (xvi) listed below:
(i) at least 25 ppmw
(ii) at least 50 ppmw
(iii) at least 75 ppmw
(iv) at least 100 ppmw
(v) at least 150 ppmw
(vi) at least 200 ppmw
(vii) at least 300 ppmw
(viii) at least 400 ppmw
(ix) at least 500 ppmw
(x) at least 750 ppmw
(xi) at least 1000 ppmw
(xii) at least 2500ppmw
(xiii) at most 5000ppmw
(xiv) at most 10000 ppmw
(xv) at most 2 %wt.
(xvi) at most 5 %wt.

Suitable friction modifiers for use herein are alkoxylated amines eg ethoxylated amines, propoxylated amines, butoxylated amines such as those commercially from Akzo-Nobel under the tradename Ethomeen and Propomeen.

Examples of suitable friction modifiers for use herein can be found in the following patent publications: US-A-7435272, US-A-6866690, WO2002/079353, WO2010/05921, WO2009/50256, WO2010/05720, WO2002/79353, WO2010/139994, WO97/45507, WO2002/02720, WO2010/012756, WO2010/012763, and PCT applications PCT/EP2010/070762 and PCT/EP2010/070762.

Examples of commercially available friction modifiers suitable for use as the second additive herein include, but are not limited to, Ultrazol 9525 commercially available from Lubrizol; Ethomeen T12, Ethomeen T12e, Ethomeen T15, Ethomeen 012, Ethomeen 015, Ethomeen T20 and Ethomeen C15 commercially available from AkzoNobel.

The first fuel additive and second fuel additive are blended together with any other additives e.g. additive performance package(s) to produce an additive blend. The additive blend is then added to a base fuel to produce a liquid fuel composition. The amount of first fuel additive in the additive blend is preferably in the range of from 0.1 to 99.8 wt%, by weight of the additive blend. The amount of second fuel additive in the additive blend is preferably in the range of from 0.1 to 99.8 wt%, by weight of the additive blend.

The amount of performance package(s)in the additive blend is preferably in the range of from 0.1 to 99.8 wt%, by weight of the additive blend.

Preferably, the amount of the performance package present in the liquid fuel composition of the present invention is in the range of 15 ppmw (parts per million by weight) to 10 %wt, based on the overall weight of the liquid fuel composition. More preferably, the amount of the performance package present in the liquid fuel composition of the present invention additionally accords with one or more of the parameters (i) to (xv) listed below:
(i) at least 100 ppmw
(ii) at least 200 ppmw
(iii) at least 300 ppmw
(iv) at least 400 ppmw
(v) at least 500 ppmw
(vi) at least 600 ppmw
(vii) at least 700 ppmw
(viii) at least 800 ppmw
(ix) at least 900 ppmw
(x) at least 1000 ppmw
(xi) at least 2500ppmw
(xii) at most 5000ppmw
(xiii) at most 10000 ppmw
(xiv) at most 2 %wt.
(xv) at most 5 %wt.

In the liquid fuel compositions of the present invention, if the base fuel used is a gasoline, then the gasoline may be any gasoline suitable for use in an internal combustion engine of the spark-ignition (petrol) type known in the art, including automotive engines as well as in other types of engine such as, for example, off road and aviation engines. The gasoline used as the base fuel in the liquid fuel composition of the present invention may conveniently also be referred to as 'base gasoline'.

Gasolines typically comprise mixtures of hydrocarbons boiling in the range from 25 to 230 °C (EN-ISO 3405), the optimal ranges and distillation curves typically varying according to climate and season of the year. The hydrocarbons in a gasoline may be derived by any means known in the art, conveniently the hydrocarbons may be derived in any known manner from straight-run gasoline, synthetically-produced aromatic hydrocarbon mixtures, thermally or catalytically cracked hydrocarbons, hydro-cracked petroleum fractions, catalytically reformed hydrocarbons or mixtures of these.

The specific distillation curve, hydrocarbon composition, research octane number (RON) and motor octane number (MON) of the gasoline are not critical.

Conveniently, the research octane number (RON) of the gasoline may be at least 80, for instance in the range of from 80 to 110, preferably the RON of the gasoline will be at least 90, for instance in the range of from 90 to 110, more preferably the RON of the gasoline will be at least 91, for instance in the range of from 91 to 105, even more preferably the RON of the gasoline will be at least 92, for instance in the range of from 92 to 103, even more preferably the RON of the gasoline will be at least 93, for instance in the range of from 93 to 102, and most preferably the RON of the gasoline will be at least 94, for instance in the range of from 94 to 100 (EN 25164); the motor octane number (MON) of the gasoline may conveniently be at least 70, for instance in the range of from 70 to 110, preferably the MON of the gasoline will be at least 75, for instance in the range of from 75 to 105, more preferably the MON of the gasoline will be at least 80, for instance in the range of from 80 to 100, most preferably the MON of the gasoline will be at least 82, for instance in the range of from 82 to 95 (EN 25163).

Typically, gasolines comprise components selected from one or more of the following groups; saturated hydrocarbons, olefinic hydrocarbons, aromatic hydrocarbons, and oxygenated hydrocarbons. Conveniently, the gasoline may comprise a mixture of saturated hydrocarbons, olefinic hydrocarbons, aromatic hydrocarbons, and, optionally, oxygenated hydrocarbons.

Typically, the olefinic hydrocarbon content of the gasoline is in the range of from 0 to 40 percent by volume based on the gasoline (ASTM D1319); preferably, the olefinic hydrocarbon content of the gasoline is in the range of from 0 to 30 percent by volume based on the gasoline, more preferably, the olefinic hydrocarbon content of the gasoline is in the range of from 0 to 20 percent by volume based on the gasoline.

Typically, the aromatic hydrocarbon content of the gasoline is in the range of from 0 to 70 percent by volume based on the gasoline (ASTM D1319), for instance the aromatic hydrocarbon content of the gasoline is in the range of from 10 to 60 percent by volume based on the gasoline; preferably, the aromatic hydrocarbon content of the gasoline is in the range of from 0 to 50 percent by volume based on the gasoline, for instance the aromatic hydrocarbon content of the gasoline is in the range of from 10 to 50 percent by volume based on the gasoline.

The benzene content of the gasoline is at most 10 percent by volume, more preferably at most 5 percent by volume, especially at most 1 percent by volume based on the gasoline.

The gasoline preferably has a low or ultra low sulphur content, for instance at most 1000 ppmw (parts per million by weight), preferably no more than 500 ppmw, more preferably no more than 100, even more preferably no more than 50 and most preferably no more than even 10 ppmw.

The gasoline also preferably has a low total lead content, such as at most 0.005 g/l, most preferably being lead free - having no lead compounds added thereto (i.e. unleaded).

When the gasoline comprises oxygenated hydrocarbons, at least a portion of non-oxygenated hydrocarbons will be substituted for oxygenated hydrocarbons. The oxygen content of the gasoline may be up to 35 percent by weight (EN 1601) (e.g. ethanol per se) based on the gasoline. For example, the oxygen content of the gasoline may be up to 25 percent by weight, preferably up to 10 percent by weight. Conveniently, the oxygenate concentration will have a minimum concentration selected from any one of 0, 0.2, 0.4, 0.6, 0.8, 1.0, and 1.2 percent by weight, and a maximum concentration selected from any one of 5, 4.5, 4.0, 3.5, 3.0, and 2.7 percent by weight.

Examples of oxygenated hydrocarbons that may be incorporated into the gasoline include alcohols, ethers, esters, ketones, aldehydes, carboxylic acids and their derivatives, and oxygen containing heterocyclic compounds. Preferably, the oxygenated hydrocarbons that may be incorporated into the gasoline are selected from alcohols (such as methanol, ethanol, propanol, 2-propanol, butanol, tert-butanol, iso-butanol and 2-butanol), ethers (preferably ethers containing 5 or more carbon atoms per molecule, e.g., methyl tert-butyl ether and ethyl tert-butyl ether) and esters (preferably esters containing 5 or more carbon atoms per molecule); a particularly preferred oxygenated hydrocarbon is ethanol.

When oxygenated hydrocarbons are present in the gasoline, the amount of oxygenated hydrocarbons in the gasoline may vary over a wide range. For example, gasolines comprising a major proportion of oxygenated hydrocarbons are currently commercially available in countries such as Brazil and U.S.A., e.g. ethanol per se and E85, as well as gasolines comprising a minor proportion of oxygenated hydrocarbons, e.g. E10 and E5. Therefore, the gasoline may contain up to 100 percent by volume oxygenated hydrocarbons. E100 fuels as used in Brazil are also included herein. Preferably, the amount of oxygenated hydrocarbons present in the gasoline is selected from one of the following amounts: up to 85 percent by volume; up to 70 percent by volume; up to 65 percent by volume; up to 30 percent by volume; up to 20 percent by volume; up to 15 percent by volume; and, up to 10 percent by volume, depending upon the desired final formulation of the gasoline. Conveniently, the gasoline may contain at least 0.5, 1.0 or 2.0 percent by volume oxygenated hydrocarbons.

Examples of suitable gasolines include gasolines which have an olefinic hydrocarbon content of from 0 to 20 percent by volume (ASTM D1319), an oxygen content of from 0 to 5 percent by weight (EN 1601), an aromatic hydrocarbon content of from 0 to 50 percent by volume (ASTM D1319) and a benzene content of at most 1 percent by volume.

Also suitable for use herein are gasoline blending components which can be derived from a biological source. Examples of such gasoline blending components can be found in WO2009/077606, WO2010/028206, WO2010/000761, European patent application nos. 09160983.4, 09176879.6, 09180904.6, and US patent application serial no. 61/312307.

Whilst not critical to the present invention, the base gasoline or the gasoline composition of the present invention may conveniently include one or more optional fuel additives, in addition to the essential fuel additive mentioned above. The concentration and nature of the optional fuel additive(s) that may be included in the base gasoline or the gasoline composition of the present invention is not critical. Non-limiting examples of suitable types of fuel additives that can be included in the base gasoline or the gasoline composition of the present invention include anti-oxidants, corrosion inhibitors, detergents, dehazers, antiknock additives, metal deactivators, valve-seat recession protectant compounds, dyes, solvents, carrier fluids, diluents and markers. Examples of suitable such additives are described generally in US Patent No. 5,855,629.

Conveniently, the fuel additives can be blended with one or more solvents to form an additive concentrate, the additive concentrate can then be admixed with the base gasoline or the gasoline composition of the present invention.

The (active matter) concentration of any optional additives present in the base gasoline or the gasoline composition of the present invention is preferably up to 1 percent by weight, more preferably in the range from 5 to 2000 ppmw, advantageously in the range of from 300 to 1500 ppmw, such as from 300 to 1000 ppmw.

As stated above, the gasoline composition may also contain synthetic or mineral carrier oils and/or solvents.

Examples of suitable mineral carrier oils are fractions obtained in crude oil processing, such as brightstock or base oils having viscosities, for example, from the SN 500 - 2000 class; and also aromatic hydrocarbons, paraffinic hydrocarbons and alkoxyalkanols. Also useful as a mineral carrier oil is a fraction which is obtained in the refining of mineral oil and is known as "hydrocrack oil" (vacuum distillate cut having a boiling range of from about 360 to 500 °C, obtainable from natural mineral oil which has been catalytically hydrogenated under high pressure and isomerized and also deparaffinized).

Examples of suitable synthetic carrier oils are: polyolefins (poly-alpha-olefins or poly(internal olefin)s), (poly)esters, (poly)alkoxylates, polyethers, aliphatic polyether amines, alkylphenol-started polyethers, alkylphenol-started polyether amines and carboxylic esters of long-chain alkanols.

Examples of suitable polyolefins are olefin polymers, in particular based on polybutene or polyisobutene (hydrogenated or nonhydrogenated).

Examples of suitable polyethers or polyetheramines are preferably compounds comprising polyoxy-C₂-C₄-alkylene moieties which are obtainable by reacting C₂-C₆₀-alkanols, C₆-C₃₀-alkanediols, mono- or di-C₂-C₃₀-alkylamines, C₁-C₃₀-alkylcyclohexanols or C₁-C₃₀-alkylphenols with from 1 to 30 mol of ethylene oxide and/or propylene oxide and/or butylene oxide per hydroxyl group or amino group, and, in the case of the polyether amines, by subsequent reductive amination with ammonia, monoamines or polyamines. Such products are described in particular in EP-A-310 875, EP-A-356 725, EP-A-700 985 and US-A-4,877,416. For example, the polyether amines used may be poly-C₂-C₆-alkylene oxide amines or functional derivatives thereof. Typical examples thereof are tridecanol butoxylates or isotridecanol butoxylates, isononylphenol butoxylates and also polyisobutenol butoxylates and propoxylates, and also the corresponding reaction products with ammonia.

Examples of carboxylic esters of long-chain alkanols are in particular esters of mono-, di- or tricarboxylic acids with long-chain alkanols or polyols, as described in particular in DE-A-38 38 918. The mono-, di- or tricarboxylic acids used may be aliphatic or aromatic acids; suitable ester alcohols or polyols are in particular long-chain representatives having, for example, from 6 to 24 carbon atoms. Typical representatives of the esters are adipates, phthalates, isophthalates, terephthalates and trimellitates of isooctanol, isononanol, isodecanol and isotridecanol, for example di-(n- or isotridecyl) phthalate.

Further suitable carrier oil systems are described, for example, in DE-A-38 26 608, DE-A-41 42 241, DE-A-43 09 074, EP-A-0 452 328 and EP-A-0 548 617, which are incorporated herein by way of reference.

Examples of particularly suitable synthetic carrier oils are alcohol-started polyethers having from about 5 to 35, for example from about 5 to 30, C₃-C₆-alkylene oxide units, for example selected from propylene oxide, n-butylene oxide and isobutylene oxide units, or mixtures thereof. Non-limiting examples of suitable starter alcohols are long-chain alkanols or phenols substituted by long-chain alkyl in which the long-chain alkyl radical is in particular a straight-chain or branched C₆-C₁₈-alkyl radical. Preferred examples include tridecanol and nonylphenol.

Further suitable synthetic carrier oils are alkoxylated alkylphenols, as described in DE-A-10 102 913.6.

Mixtures of mineral carrier oils, synthetic carrier oils, and mineral and synthetic carrier oils may also be used.

Any solvent and optionally co-solvent suitable for use in fuels may be used. Examples of suitable solvents for use in fuels include: non-polar hydrocarbon solvents such as kerosene, heavy aromatic solvent ("solvent naphtha heavy", "Solvesso 150"), toluene, xylene, paraffins, petroleum, white spirits, those sold by Shell companies under the trademark "SHELLSOL", and the like. Examples of suitable co-solvents include: polar solvents such as esters and, in particular, alcohols (e.g. t-butanol, i-butanol, hexanol, 2-ethylhexanol, 2-propyl heptanol, decanol, isotridecanol, butyl glycols, and alcohol mixtures such as those sold by Shell companies under the trade mark "LINEVOL", especially LINEVOL 79 alcohol which is a mixture of C₇₋₉ primary alcohols, or a C₁₂₋₁₄ alcohol mixture which is commercially available).

Dehazers/demulsifiers suitable for use in liquid fuels are well known in the art. Non-limiting examples include glycol oxyalkylate polyol blends (such as sold under the trade designation TOLAD™ 9312), alkoxylated phenol formaldehyde polymers, phenol/formaldehyde or C₁₋₁₈ alkylphenol/-formaldehyde resin oxyalkylates modified by oxyalkylation with C₁₋₁₈ epoxides and diepoxides (such as sold under the trade designation TOLAD™ 9308), and C₁₋₄ epoxide copolymers cross-linked with diepoxides, diacids, diesters, diols, diacrylates, dimethacrylates or diisocyanates, and blends thereof. The glycol oxyalkylate polyol blends may be polyols oxyalkylated with C₁₋₄ epoxides. The C₁₋₁₈ alkylphenol phenol/-formaldehyde resin oxyalkylates modified by oxyalkylation with C₁₋₁₈ epoxides and diepoxides may be based on, for example, cresol, t-butyl phenol, dodecyl phenol or dinonyl phenol, or a mixture of phenols (such as a mixture of t-butyl phenol and nonyl phenol). The dehazer should be used in an amount sufficient to inhibit the hazing that might otherwise occur when the gasoline without the dehazer contacts water, and this amount will be referred to herein as a "haze-inhibiting amount." Generally, this amount is from about 0.1 to about 20 ppmw (e.g. from about 0.1 to about 10 ppm), more preferably from 1 to 15 ppmw, still more preferably from 1 to 10 ppmw, advantageously from 1 to 5 ppmw based on the weight of the gasoline.

Further customary additives for use in gasolines are corrosion inhibitors, for example based on ammonium salts of organic carboxylic acids, said salts tending to form films, or of heterocyclic aromatics for nonferrous metal corrosion protection; antioxidants or stabilizers, for example based on amines such as phenyldiamines, e.g. p-phenylenediamine, N,N'-di-sec-butyl-p-phenyldiamine, dicyclohexylamine or derivatives thereof or of phenols such as 2,4-di-tert-butylphenol or 3,5-di-tert-butyl-4-hydroxy-phenylpropionic acid; anti-static agents; metallocenes such as ferrocene; methylcyclopentadienylmanganese tricarbonyl; lubricity additives, such as certain fatty acids, alkenylsuccinic esters, bis(hydroxyalkyl) fatty amines, hydroxyacetamides or castor oil; and also dyes (markers). Amines may also be added, if appropriate, for example as described in WO 03/076554. Optionally anti valve seat recession additives may be used such as sodium or potassium salts of polymeric organic acids.

The gasoline compositions herein can also comprise a detergent additive. Suitable detergent additives include those disclosed in WO2009/50287.

Preferred detergent additives for use in the gasoline composition herein typically have at least one hydrophobic hydrocarbon radical having a number-average molecular weight (Mn) of from 85 to 20 000 and at least one polar moiety selected from:
(A1) mono- or polyamino groups having up to 6 nitrogen atoms, of which at least one nitrogen atom has basic properties;
(A6) polyoxy-C₂- to -C₄-alkylene groups which are terminated by hydroxyl groups, mono- or polyamino groups, in which at least one nitrogen atom has basic properties, or by carbamate groups;
(A8) moieties derived from succinic anhydride and having hydroxyl and/or amino and/or amido and/or imido groups; and/or
(A9) moieties obtained by Mannich reaction of substituted phenols with aldehydes and mono- or polyamines.

The hydrophobic hydrocarbon radical in the above detergent additives, which ensures the adequate solubility in the base fluid, has a number-average molecular weight (Mn) of from 85 to 20 000, especially from 113 to 10 000, in particular from 300 to 5000. Typical hydrophobic hydrocarbon radicals, especially in conjunction with the polar moieties (A1), (A8) and (A9), include polyalkenes (polyolefins), such as the polypropenyl, polybutenyl and polyisobutenyl radicals each having Mn of from 300 to 5000, preferably from 500 to 2500, more preferably from 700 to 2300, and especially from 700 to 1000.

Non-limiting examples of the above groups of detergent additives include the following:
Additives comprising mono- or polyamino groups (A1) are preferably polyalkenemono- or polyalkenepolyamines based on polypropene or conventional (i.e. having predominantly internal double bonds) polybutene or polyisobutene having Mn of from 300 to 5000. When polybutene or polyisobutene having predominantly internal double bonds (usually in the beta and gamma position) are used as starting materials in the preparation of the additives, a possible preparative route is by chlorination and subsequent amination or by oxidation of the double bond with air or ozone to give the carbonyl or carboxyl compound and subsequent amination under reductive (hydrogenating) conditions. The amines used here for the amination may be, for example, ammonia, monoamines or polyamines, such as dimethylaminopropylamine, ethylenediamine, diethylenetriamine, triethylenetetramine or tetraethylenepentamine. Corresponding additives based on polypropene are described in particular in WO-A-94/24231.

Further preferred additives comprising monoamino groups (A1) are the hydrogenation products of the reaction products of polyisobutenes having an average degree of polymerization of from 5 to 100, with nitrogen oxides or mixtures of nitrogen oxides and oxygen, as described in particular in WO-A-97/03946.

Further preferred additives comprising monoamino groups (A1) are the compounds obtainable from polyisobutene epoxides by reaction with amines and subsequent dehydration and reduction of the amino alcohols, as described in particular in DE-A-196 20 262.

Additives comprising polyoxy-C₂-C₄-alkylene moieties (A6) are preferably polyethers or polyetheramines which are obtainable by reaction of C₂- to C₆₀-alkanols, C₆- to C₃₀-alkanediols, mono- or di-C₂-C₃₀-alkylamines, C₁-C₃₀-alkylcyclohexanols or C₁-C₃₀-alkylphenols with from 1 to 30 mol of ethylene oxide and/or propylene oxide and/or butylene oxide per hydroxyl group or amino group and, in the case of the polyether-amines, by subsequent reductive amination with ammonia, monoamines or polyamines. Such products are described in particular in EP-A-310 875, EP-A-356 725, EP-A-700 985 and US-A-4 877 416. In the case of polyethers, such products also have carrier oil properties. Typical examples of these are tridecanol butoxylates, isotridecanol butoxylates, isononylphenol butoxylates and polyisobutenol butoxylates and propoxylates and also the corresponding reaction products with ammonia.

Additives comprising moieties derived from succinic anhydride and having hydroxyl and/or amino and/or amido and/or imido groups (A8) are preferably corresponding derivatives of polyisobutenylsuccinic anhydride which are obtainable by reacting conventional or highly reactive polyisobutene having Mn of from 300 to 5000 with maleic anhydride by a thermal route or via the chlorinated polyisobutene. Of particular interest are derivatives with aliphatic polyamines such as ethylenediamine, diethylenetriamine, triethylenetetramine or tetraethylenepentamine. Such additives are described in particular in US-A-4 849 572.

Additives comprising moieties obtained by Mannich reaction of substituted phenols with aldehydes and mono- or polyamines (A9) are preferably reaction products of polyisobutene-substituted phenols with formaldehyde and mono- or polyamines such as ethylenediamine, diethylenetriamine, triethylenetetramine, tetraethylenepentamine or dimethylaminopropylamine. The polyisobutenyl-substituted phenols may stem from conventional or highly reactive polyisobutene having Mn of from 300 to 5000. Such "polyisobutene-Mannich bases" are described in particular in EP-A-831 141.

Preferably, the detergent additive used in the gasoline compositions of the present invention contains at least one nitrogen-containing detergent, more preferably at least one nitrogen-containing detergent containing a hydrophobic hydrocarbon radical having a number average molecular weight in the range of from 300 to 5000. Preferably, the nitrogen-containing detergent is selected from a group comprising polyalkene monoamines, polyetheramines, polyalkene Mannich amines and polyalkene succinimides. Conveniently, the nitrogen-containing detergent may be a polyalkene monoamine.

In the liquid fuel compositions, if the base fuel used is a diesel fuel, then the diesel fuel used as the base fuel includes diesel fuels for use in automotive compression ignition engines, as well as in other types of engine such as for example off road, marine, railroad and stationary engines. The diesel fuel used as the base fuel in the liquid fuel composition may conveniently also be referred to as 'diesel base fuel'.

The diesel base fuel may itself comprise a mixture of two or more different diesel fuel components, and/or be additivated as described below.

Such diesel fuels will contain one or more base fuels which may typically comprise liquid hydrocarbon middle distillate gas oil(s), for instance petroleum derived gas oils. Such fuels will typically have boiling points within the usual diesel range of 150 to 400°C, depending on grade and use. They will typically have a density from 750 to 1000 kg/m³, preferably from 780 to 860 kg/m³, at 15°C (e.g. ASTM D4502 or IP 365) and a cetane number (ASTM D613) of from 35 to 120, more preferably from 40 to 85. They will typically have an initial boiling point in the range 150 to 230°C and a final boiling point in the range 290 to 400°C. Their kinematic viscosity at 40°C (ASTM D445) might suitably be from 1.2 to 4.5 mm²/s.

An example of a petroleum derived gas oil is a Swedish Class 1 base fuel, which will have a density from 800 to 820 kg/m³ at 15°C (SS-EN ISO 3675, SS-EN ISO 12185), a T95 of 320°C or less (SS-EN ISO 3405) and a kinematic viscosity at 40°C (SS-EN ISO 3104) from 1.4 to 4.0 mm²/s, as defined by the Swedish national specification EC1.

Optionally, non-mineral oil based fuels, such as biofuels or Fischer-Tropsch derived fuels, may also form or be present in the diesel fuel. Such Fischer-Tropsch fuels may for example be derived from natural gas, natural gas liquids, petroleum or shale oil, petroleum or shale oil processing residues, coal or biomass.

The amount of Fischer-Tropsch derived fuel used in the diesel fuel may be from 0% to 100%v of the overall diesel fuel, preferably from 5% to 100%v, more preferably from 5% to 75%v. It may be desirable for such a diesel fuel to contain 10%v or greater, more preferably 20%v or greater, still more preferably 30%v or greater, of the Fischer-Tropsch derived fuel. It is particularly preferred for such diesel fuels to contain 30 to 75%v, and particularly 30 to 70%v, of the Fischer-Tropsch derived fuel. The balance of the diesel fuel is made up of one or more other diesel fuel components.

Such a Fischer-Tropsch derived fuel component is any fraction of the middle distillate fuel range, which can be isolated from the (optionally hydrocracked) Fischer-Tropsch synthesis product. Typical fractions will boil in the naphtha, kerosene or gas oil range. Preferably, a Fischer-Tropsch product boiling in the kerosene or gas oil range is used because these products are easier to handle in for example domestic environments. Such products will suitably comprise a fraction larger than 90 wt% which boils between 160 and 400°C, preferably to about 370°C. Examples of Fischer-Tropsch derived kerosene and gas oils are described in EP-A-0583836, WO-A-97/14768, WO-A-97/14769, WO-A-00/11116, WO-A-00/11117, WO-A-01/83406, WO-A-01/83648, WO-A-01/83647, WO-A-01/83641, WO-A-00/20535, WO-A-00/20534, EP-A-1101813, US-A-5766274, US-A-5378348, US-A-5888376 and US-A-6204426.

The Fischer-Tropsch product will suitably contain more than 80 wt% and more suitably more than 95 wt% iso and normal paraffins and less than 1 wt% aromatics, the balance being naphthenics compounds. The content of sulphur and nitrogen will be very low and normally below the detection limits for such compounds. For this reason the sulphur content of a diesel fuel composition containing a Fischer-Tropsch product may be very low.

The diesel fuel composition preferably contains no more than 5000ppmw sulphur, more preferably no more than 500ppmw, or no more than 350ppmw, or no more than 150ppmw, or no more than 100ppmw, or no more than 70ppmw, or no more than 50ppmw, or no more than 30ppmw, or no more than 20ppmw, or most preferably no more than 10ppmw sulphur.

Other diesel fuel components include the so-called "biofuels" which derive from biological materials. Examples include fatty acid alkyl esters (FAAE). Examples of such components can be found in WO2008/135602.

The diesel base fuel may itself be additivated (additive-containing) or unadditivated (additive-free). If additivated, e.g. at the refinery, it will contain minor amounts of one or more additives selected for example from anti-static agents, pipeline drag reducers, flow improvers (e.g. ethylene/vinyl acetate copolymers or acrylate/maleic anhydride copolymers), lubricity additives, antioxidants and wax anti-settling agents.

Detergent-containing diesel fuel additives are known and commercially available. Such additives may be added to diesel fuels at levels intended to reduce, remove, or slow the build-up of engine deposits.

Examples of detergents suitable for use in diesel fuel additives for the present purpose include polyolefin substituted succinimides or succinamides of polyamines, for instance polyisobutylene succinimides or polyisobutylene amine succinamides, aliphatic amines, Mannich bases or amines and polyolefin (e.g. polyisobutylene) maleic anhydrides. Succinimide dispersant additives are described for example in GB-A-960493, EP-A-0147240, EP-A-0482253, EP-A-0613938, EP-A-0557516 and WO-A-98/42808. Particularly preferred are polyolefin substituted succinimides such as polyisobutylene succinimides.

The diesel fuel additive mixture may contain other components in addition to the detergent. Examples are lubricity enhancers; dehazers, e.g. alkoxylated phenol formaldehyde polymers; anti-foaming agents (e.g. polyether-modified polysiloxanes); ignition improvers (cetane improvers) (e.g. 2-ethylhexyl nitrate (EHN), cyclohexyl nitrate, di-tert-butyl peroxide and those disclosed in US-A-4208190 at column 2, line 27 to column 3, line 21); anti-rust agents (e.g. a propane-1,2-diol semi-ester of tetrapropenyl succinic acid, or polyhydric alcohol esters of a succinic acid derivative, the succinic acid derivative having on at least one of its alpha-carbon atoms an unsubstituted or substituted aliphatic hydrocarbon group containing from 20 to 500 carbon atoms, e.g. the pentaerythritol diester of polyisobutylene-substituted succinic acid); corrosion inhibitors; reodorants; anti-wear additives; anti-oxidants (e.g. phenolics such as 2,6-di-tert-butylphenol, or phenylenediamines such as N,N'-di-sec-butyl-p-phenylenediamine); metal deactivators; combustion improvers; static dissipator additives; cold flow improvers; and wax anti-settling agents.

The diesel fuel additive mixture may contain a lubricity enhancer, especially when the diesel fuel composition has a low (e.g. 500 ppmw or less) sulphur content. In the additivated diesel fuel composition, the lubricity enhancer is conveniently present at a concentration of less than 1000 ppmw, preferably between 50 and 1000 ppmw, more preferably between 70 and 1000 ppmw. Suitable commercially available lubricity enhancers include ester- and acid-based additives. Other lubricity enhancers are described in the patent literature, in particular in connection with their use in low sulphur content diesel fuels, for example in:
- the paper by Danping Wei and H.A. Spikes, "The Lubricity of Diesel Fuels", Wear, III (1986) 217-235;
- WO-A-95/33805 - cold flow improvers to enhance lubricity of low sulphur fuels;
- US-A-5490864 - certain dithiophosphoric diester-dialcohols as anti-wear lubricity additives for low sulphur diesel fuels; and
- WO-A-98/01516 - certain alkyl aromatic compounds having at least one carboxyl group attached to their aromatic nuclei, to confer anti-wear lubricity effects particularly in low sulphur diesel fuels.

It may also be preferred for the diesel fuel composition to contain an anti-foaming agent, more preferably in combination with an anti-rust agent and/or a corrosion inhibitor and/or a lubricity enhancing additive.

Unless otherwise stated, the (active matter) concentration of each such optional additive component in the additivated diesel fuel composition is preferably up to 10000 ppmw, more preferably in the range from 0.1 to 1000 ppmw, advantageously from 0.1 to 300 ppmw, such as from 0.1 to 150 ppmw.

The (active matter) concentration of any dehazer in the diesel fuel composition will preferably be in the range from 0.1 to 20 ppmw, more preferably from 1 to 15 ppmw, still more preferably from 1 to 10 ppmw, and especially from 1 to 5 ppmw. The (active matter) concentration of any ignition improver present will preferably be 2600 ppmw or less, more preferably 2000 ppmw or less, even more preferably 300 to 1500 ppmw. The (active matter) concentration of any detergent in the diesel fuel composition will preferably be in the range from 5 to 1500 ppmw, more preferably from 10 to 750 ppmw, most preferably from 20 to 500 ppmw.

In the case of a diesel fuel composition, for example, the fuel additive mixture will typically contain a detergent, optionally together with other components as described above, and a diesel fuel-compatible diluent, which may be a mineral oil, a solvent such as those sold by Shell companies under the trade mark "SHELLSOL", a polar solvent such as an ester and, in particular, an alcohol, e.g. hexanol, 2-ethylhexanol, decanol, isotridecanol and alcohol mixtures such as those sold by Shell companies under the trade mark "LINEVOL", especially LINEVOL 79 alcohol which is a mixture of C₇₋₉ primary alcohols, or a C₁₂₋₁₄ alcohol mixture which is commercially available.

The total content of the additives in the diesel fuel composition may be suitably between 0 and 10000 ppmw and preferably below 5000 ppmw.

In the above, amounts (concentrations, % vol, ppmw, % wt) of components are of active matter, i.e. exclusive of volatile solvents/diluent materials.

The liquid fuel composition is produced by admixing the at least one essential fuel additive with a base fuel suitable for use in an internal combustion engine. If the base fuel to which the essential fuel additive is admixed is a gasoline, then the liquid fuel composition produced is a gasoline composition; likewise, if the base fuel to which the fuel additive is admixed is a diesel fuel, then the liquid fuel composition produced is a diesel fuel composition.

It has surprisingly been found that the use of a fuel additive having a kinematic viscosity at 100°C of 27 cSt or less and a NOACK volatility at 250°C of 100 %wt, preferably 20 wt% or less, and a friction modifier in liquid fuel compositions provides benefits in terms of improved fuel economy of an internal combustion engine being fuelled by the liquid fuel composition containing said additive, in particular when the liquid fuel composition of the present invention is a gasoline composition, relative to the internal combustion engine being fuelled by the liquid base fuel.

The present invention therefore provides a method of improving the fuel economy performance of a liquid base fuel suitable for use in an internal combustion engine, comprising admixing at least one fuel additive having a kinematic viscosity at 100°C of 27 cSt or less and a NOACK volatility at 250°C of 100 %wt, preferably 20 wt% or less, and at least one friction modifier with a major portion of a liquid base fuel suitable for use in an internal combustion engine.

Additionally, the use of the at least one fuel additive having a kinematic viscosity at 100°C of 27 cSt or less and a NOACK volatility at 250°C of 100 %wt, preferably 20 wt% or less, in combination with a friction modifier in liquid fuel compositions can also provide benefits in terms improving the lubricant performance of an internal combustion engine being fuelled by the liquid fuel composition of the present invention relative to the internal combustion engine being fuelled by the liquid base fuel.

Therefore, also described herein is a method of improving the performance of the lubricant of an internal combustion engine, said method comprising fuelling an internal combustion engine containing the engine lubricant with a liquid fuel composition according to the present invention.

Additionally, the use of the at least one fuel additive having a kinematic viscosity at 100°C of 27 cSt or less and a NOACK volatility at 250°C of 100 %wt, preferably 20 wt% or less, and at least one friction modifier in liquid fuel compositions can also provide benefits in terms of improving the fuel economy performance of a lubricant of an internal combustion engine being fuelled by the liquid fuel composition of the present invention.

Therefore, the present invention provides a method of improving the fuel economy performance of a lubricant of an internal combustion engine, said method comprising fuelling the internal combustion engine containing the lubricant with a liquid fuel composition comprising:
- a base fuel suitable for use in an internal combustion engine, wherein the base fuel is a gasoline or a diesel fuel; and
- at least one first fuel additive having:
   (i) a kinematic viscosity at 100°C of 27 cSt or less; and
   (ii) a NOACK volatility at 250°C of 100 %wt, preferably 20 %wt or less; and
- at least one friction modifier, wherein the one or more friction modifiers is selected from alkoxylated amines;
wherein the first fuel additive is PAO-2, and wherein the liquid fuel composition is a gasoline composition.

### Lubricating Oil

Lubricating oil compositions herein contain a lubricating oil as the base fluid, and are suitable for use as an engine crank case lubricant.

The total amount of lubricating oil incorporated in the lubricating oil composition is at least 60 percent by weight, preferably in the range of from 60 to 92 percent by weight, more preferably in the range of from 75 to 90 percent by weight and most preferably in the range of from 75 to 88 percent by weight, with respect to the total weight of the lubricating oil composition.

There are no particular limitations regarding the lubricating oil used in the lubricating oil composition, and various conventional known mineral oils and synthetic oils may be conveniently used.

The lubricating oil used in the lubricating oil composition may conveniently comprise mixtures of one or more mineral oils and/or one or more synthetic oils.

Mineral oils include liquid petroleum oils and solvent-treated or acid-treated mineral lubricating oil of the paraffinic, naphthenic, or mixed paraffinic/naphthenic type which may be further refined by hydrofinishing processes and/or dewaxing.

Naphthenic lubricating oils have low viscosity index (VI) (generally 40-80) and a low pour point. Such lubricating oils are produced from feedstocks rich in naphthenes and low in wax content and are used mainly for lubricants in which colour and colour stability are important, and VI and oxidation stability are of secondary importance.

Paraffinic lubricating oils have higher VI (generally >95) and a high pour point. Said lubricating oils are produced from feedstocks rich in paraffins, and are used for lubricants in which VI and oxidation stability are important.

Fischer-Tropsch derived lubricating oils may be conveniently used in the lubricating oil composition, for example, the Fischer-Tropsch derived lubricating oils disclosed in EP-A-776959, EP-A-668342, WO-A-97/21788, WO-00/15736, WO-00/14188, WO-00/14187, WO-00/14183, WO-00/14179, WO-00/08115, WO-99/41332, EP-1029029, WO-01/18156 and WO-01/57166.

Synthetic processes enable molecules to be built from simpler substances or to have their structures modified to give the precise properties required.

Synthetic lubricating oils include hydrocarbon oils such as olefin oligomers (PAOs), dibasic acids esters, polyol esters, and dewaxed waxy raffinate. Synthetic hydrocarbon base oils sold by the Royal Dutch/Shell Group of Companies under the designation "XHVI" (trade mark) may be conveniently used.

Preferably, the lubricating oil is constituted from mineral oils and/or synthetic oils which contain more than 80% wt of saturates, preferably more than 90 percent by weight, as measured according to ASTM D2007.

It is further preferred that the lubricating oil contains less than 1.0 percent by weight, preferably less than 0.1 percent by weight of sulphur, calculated as elemental sulphur and measured according to ASTM D2622, ASTM D4294, ASTM D4927 or ASTM D3120.

Preferably, the viscosity index of the lubricating oil, is more than 80, more preferably more than 120, as measured according to ASTM D2270.

Preferably, the lubricating oil has a kinematic viscosity in the range of from 2 to 80 mm²/s at 100 °C, more preferably in the range of from 3 to 70 mm²/s, most preferably in the range of from 4 to 50 mm²/s.

The total amount of phosphorus in the lubricating oil is preferably in the range of from 0.04 to 0.1 percent by weight, more preferably in the range of from 0.04 to 0.09 percent by weight and most preferably in the range of from 0.045 to 0.09 percent by weight, based on total weight of the lubricating oil.

The lubricating oil preferably has a sulphated ash content of not greater than 1.0 percent by weight, more preferably not greater than 0.75 percent by weight and most preferably not greater than 0.7 percent by weight, based on the total weight of the lubricating oil.

The lubricating oil composition preferably has a sulphur content of not greater than 1.2 percent by weight, more preferably not greater than 0.8 percent by weight and most preferably not greater than 0.2 percent by weight, based on the total weight of the lubricating oil lubricating oil composition.

The lubricating oil composition may further comprise additives such as anti-oxidants, anti-wear additives, detergents, dispersants, friction modifiers, viscosity index improvers, pour point depressants, corrosion inhibitors, defoaming agents and seal fix or seal compatibility agents.

Antioxidants that may be conveniently used include those selected from the group of aminic antioxidants and/or phenolic antioxidants.

In a preferred embodiment, said antioxidants are present in an amount in the range of from 0.1 to 5.0 percent by weight, more preferably in an amount in the range of from 0.3 to 3.0 percent by weight, and most preferably in an amount of in the range of from 0.5 to 1.5 percent by weight, based on the total weight of the lubricating oil composition.

The lubricating oil composition may conveniently contain a single zinc dithiophosphate or a combination of two or more zinc dithiophosphates as anti-wear additives, the or each zinc dithiophosphate being selected from zinc dialkyl-, diaryl- or alkylaryl-dithiophosphates.

The lubricating oil composition may generally contain in the range of from 0.4 to 1.0 percent by weight of zinc dithiophosphate, based on total weight of the lubricating oil composition.

Additional or alternative anti-wear additives may be conveniently used in the lubricating oil composition herein.

Suitable alternative anti-wear additives include boron-containing compounds such as borate esters, borated fatty amines, borated epoxides, alkali metal (or mixed alkali or alkaline earth metal) borates and borated overbased metal salts. Said boron-containing anti-wear additives may be conveniently added to the lubricating oil in an amount in the range of from 0.1 to 3.0 percent by weight, based on the total weight of lubricating oil composition.

Typical detergents that may be used in the lubricating oil composition include one or more salicylate and/or phenate and/or sulphonate detergents.

However, as metal organic and inorganic base salts which are used as detergents can contribute to the sulphated ash content of a lubricating oil composition, in a preferred embodiment of the present invention, the amounts of such additives are minimised.

Furthermore, in order to maintain a low sulphur level, salicylate detergents are preferred.

Thus, in a preferred embodiment, the lubricating oil composition may contain one or more salicylate detergents.

In order to maintain the total sulphated ash content of the lubricating oil composition at a level of preferably not greater than 1.0 percent by weight, more preferably at a level of not greater than 0.75 percent by weight and most preferably at a level of not greater than 0.7 percent by weight, based on the total weight of the lubricating oil composition, said detergents are preferably used in amounts in the range of 0.05 to 12.5 percent by weight, more preferably from 1.0 to 9.0 percent by weight and most preferably in the range of from 2.0 to 5.0 percent by weight, based on the total weight of the lubricating oil composition.

Furthermore, it is preferred that said detergents, independently, have a TBN (total base number) value in the range of from 10 to 500 mg.KOH/g, more preferably in the range of from 30 to 350 mg.KOH/g and most preferably in the range of from 50 to 300 mg.KOH/g, as measured by ISO 3771.

The lubricating oil compositions may additionally contain an ash-free dispersant which is preferably admixed in an amount in the range of from 5 to 15 percent by weight, based on the total weight of the lubricating oil composition.

Examples of ash-free dispersants which may be used include the polyalkenyl succinimides and polyalkenyl succininic acid esters disclosed in Japanese Patent Nos. 1367796, 1667140, 1302811 and 1743435. Preferred dispersants include borated succinimides.

Examples of viscosity index improvers which may conveniently used in the lubricating oil composition include the styrene-butadiene copolymers, styreneisoprene stellate copolymers and the polymethacrylate copolymer and ethylene-propylene copolymers. Such viscosity index improvers may be conveniently employed in an amount in the range of from 1 to 20 percent by weight, based on the total weight of the lubricating oil composition.

Polymethacrylates may be conveniently employed in the lubricating oil compositions as effective pour point depressants.

Furthermore, compounds such as alkenyl succinic acid or ester moieties thereof, benzotriazole-based compounds and thiodiazole-based compounds may be conveniently used in the lubricating oil composition as corrosion inhibitors.

Compounds such as polysiloxanes, dimethyl polycyclohexane and polyacrylates may be conveniently used in the lubricating oil composition as defoaming agents.

Compounds which may be conveniently used in the lubricating oil composition as seal fix or seal compatibility agents include, for example, commercially available aromatic esters.

The present invention will be further understood from the following examples. Unless otherwise stated, all amounts and concentrations disclosed in the examples are based on weight of the fully formulated fuel composition.

### Examples

### Examples 1 to 4

The composition and properties of a number of commercially available components that can be used as first fuel additive and second fuel additive are given below. Certain of these components are used in Examples 1 to 4.

Durasyn 165, a PAO-5 commercially available from INEOS Oligomers.

Durasyn 162, a PAO-2 commercially available from INEOS Oligomers.

Priolube 3970, a C7-C9 ester of trimethylolpropane commercially available from Croda Europe Limited.

FM10 - this is a reaction product of oleic acid and aminoethylethanolamine having a 3:1 molar ratio as per Example 4 of WO2009/50287.

Ethomeen T12e, an ethoxylated amine produced from tallowamine with an average 2 moles of ethyleneoxide, commercially available from AkzoNobel.

FM11 - this is the reaction product of C8-C18 fatty acids and C18 unsaturated fatty acids with diethanolamine and propylene oxide (as disclosed in WO2010/05720).

| *Trade Name* | *Supplier* | *Chemistry* | *KV 100*°C *ASTM D445 (cSt)* | *NOACK 250*°C *ASTM D5800 (%wt)* |
|---|---|---|---|---|
| Durasyn 162 | INEOS Oligomers | Poly Alpha Olefin 2 | 2.1 | 99 |
| Durasyn 164 | INEOS Oligomers | Poly Alpha Olefin 4 | 4.1 | 14 |
| Durasyn 166 | INEOS Oligomers | Poly Alpha Olefin 6 | 6.1 | 9 |
| Durasyn 168 | INEOS Oligomers | Poly Alpha Olefin 8 | 7.77 | 3.13 |
| Synfluid PAO 5 | Chevron Corporation | Poly Alpha Olefin 5 | 5.1 | 5.8 |
| Durasyn 165 | INEOS Oligomers | Poly Alpha Olefin 5 | 5.1 | 5.5 |
| Durasyn 125 | INEOS Oligomers | Poly Alpha Olefin 5 | 5.1 | 5.5 |
| Priolube 3970 | Croda Europe Limited | TMP Cocoate Ester | 4.4 | 4.5 |
| Priolube1858 | Croda Europe Limited | Diisodecyl Azelate Ester | 4.5 | 7.2 |
| Synative ES EHO | Cognis Gmbh | 2-Ethylhexyl Oleate Ester | 2.8 | 20 |
| Synative ES 3824 | Cognis Gmbh | Neopentyl Glycol Cocoate/C8-10 Ester | 2.5 | 7.6 |

### Example 1

Products 1-18 were tested using a modified HFRR (ISO 12156) method to allow testing in gasoline. The lubricity of the gasoline compositions was determined by using a modified HFRR test. The modified HFRR test is based on ISO 12156-1 using a PCS Instruments HFRR supplemented with the PCS Instruments Gasoline Conversion Kit, and using a fluid volume of 15.0 ml (+/- 0.2 ml), a fluid temperature of 25.0 °C (+/- 1 °C), and wherein a PTFE cover is used to cover the test sample in order to minimise evaporation.

The additives were tested at 200mg/L in an unleaded gasoline meeting EN228 specifications, containing no ethanol (E0). Lower lubricity and friction coefficient results are indications of better friction modification effects and indicates better fuel economy. This is shown by Friction modifiers d to j in Table 1 below.

**Table 1**

| | *Test molecule* | *Lubricity result (microns) average* | *Friction Coefficient average* |
|---|---|---|---|
| Base Fuel | Unleaded gasoline ULG95, E0 | 872.5 | 0.641 |
| Detergent a (type A8) | PIB Succinimide detergent | 720 | 0.448 |
| Detergent b (type A6) | Poly ether amine detergent | 887 | 0.632 |
| Detergent c (type A1) | PIBAmine detergent | 871 | 0.812 |
| Friction modifier d | FM11 | 534.5 | 0.284 |
| Friction modifier e | Kerocom K3561 | 385.5 | 0.212 |
| Friction modifier f | FM10 | 401 | 0.246 |
| Friction modifier g | Ultrazol 9525 | 549.5 | 0.281 |
| Friction modifier h | Priolube 1407 | 308 | 0.196 |
| Friction modifier i | Ethomeen T12e | 481 | 0.287 |
| Friction modifier j | Ethomeen 015 | 697 | 0.344 |
| VCA k | PAO 2 (Durasyn 162) | 879.5 | 0.683 |
| VCA 1 | PAO 4 (Durasyn 164) | 872.5 | 0.657 |
| VCA m | PAO 5 (Synfluid PAO 5) | 880.5 | 0.729 |
| VCA n | PAO 8 (Durasyn 168) | 870.5 | 0.668 |
| VCA o | Priolube 3970 | 890 | 0.717 |
| VCA p | Synative ES 3824 | 869 | 0.636 |
| VCA q | Priolube1858 | 844 | 0.771 |
| VCA r | SYNATIVE ES EHO | 857 | 0.636 |

This example shows that molecules designed for detergent performance (a-c) do not show friction modification performance, and molecules designed for VCA performance (k-r) do not show friction modification performance.

### Example 2

3 vehicles of Five models (see Table 2) completed 10,000 miles of on-road mixed driving style mileage accumulation. The vehicles used standard ULG95, an ethanol-free base fuel that meets standard specification EN 228. In each case the base fuel was pre-treated with the same commercial detergent additive package, and each fuel additionally contained a test additive at a concentration detailed in Table 3.

**Table 2**

| |
|---|
| VW Golf 1.6ltr S |
| Ford Mondeo 2.0ltr Edge |
| Mitsubishi Lancer 1.8ltr GS2 |
| GM Zafira 1.6 16v Active |
| Honda Civic 1.8 SE |

**Table 3: Test Fuel Composition**

| | *(Test) Fuel* | *(Test) Fuel* | *(Test) Fuel* |
|---|---|---|---|
| Base Fuel | EN228 ULG95 | EN228 ULG95 | EN228 ULG95 |
| Lubricant | Shell Helix HX7 SAE 10W-40 | Shell Helix HX7 SAE 5W-30 | Shell Helix HX7 SAE 5W-30 |
| Detergent Package | Commercial Package | Commercial Package | Commercial Package |
| Test Additives | PAO5 at 1000ppmw | CH-2C at 200ppmw | CH-5 at 200ppmw |
| Average Test Additive concentration in lubricant after 10,000 miles | 6.1%m/m | 1.6%m/m | 1.6%m/m |
| Average fuel economy (steady state) benefit across 5 models | 0.74% | 0.84% | 0.54% |

Fuel consumption was measured at steady state conditions (32km/h 2^{nd} gear). Duplicate emissions tests were carried out on each vehicle at 10,000 miles.

Test additive concentration in the lubricant after 10,000 miles was determined by either GC - gas chromatography (PAO5) or NMR (CH-2C and CH-5).

Friction modifiers CH-2C and CH-5 are commercially available from Shanghai Sanzheng Polymer Company.

PAO-5 is Synfluid PAO 5 commercially available from Chevron Philips.

### Example 3

Two fuels were tested to study additive transfer into a lubricant.

A test was run on a pair of Ford Focus ST-2 2.5ltr cars with about 22,000miles on the odometer. The lubricant used was Helix Ultra Extra 5W-30 commercially available from Shell Lubricants. The base fuel was an EN228 gasoline base fuel. The cars were run on additised fuel containing detergent package, friction modifier and viscosity control additive.

The lubricant was sampled at the start of test and end of a 12,000 mile accumulation on a high speed cycle chassis dynameter programme. No oil top ups were permitted. The amount of additive in the lubricant, at the start and accumulated by the end of test, was measured by GC for the POA5 and Priolube 3970 or LC-MS (liquid chromatography - mass spectrometry) for FM10.

**Table 4**

| *Test* | *Friction modifier* | *Concentration in fuel* | *Increase in Concentration in lubricant after test* | *Viscosity control additive* | *Concentration in fuel* | *Increase in Concentration in lubricant* after test |
|---|---|---|---|---|---|---|
| 1 | FM10 | 225ppmw | 2000ppmw | Synfluid POA5 | 1000ppmw | 4.5%m/m |
| 2 | FM10 | 225ppmw | 2100ppmw | Priolube3970 | 1000ppmw | 5.1%m/m |

Examples 2 and 3 confirm that both friction modifiers and VCA chemistry can be transferred from the fuel to the lubricant, and, from Example 2, provide fuel economy benefits.

### Example 4

The fuel consumption and fuel economy benefit of various additives dosed directly into the lubricant in the engine sump to mimic the accumulation of additives and additive combinations, as shown to occur in Example 3, was compared with that of an undosed lubricant by using a bench engine test. The test used a Ford Zetec 1.988 litre 4-cylinder inline DOHC petrol engine. The fuel used was an EN228 Low Sulphur E5 Gasoline. The lubricant used was Shell Helix 5W-30 or Shell Helix Plus 10W40.

The engine was clean and free from abnormal levels of Inlet Valve Deposits (IVDs) and Combustion Chamber Deposits (CCDs). The test was based on the continuous repetition of the set of speed/load points (test cycle). The cycle was repeated over a total period of approximately 21 hours (16 hours overnight lubricant degreening and 5 hours fuel consumption measurements) with scheduled breaks for the acquisition of lubricant samples and the injection of the additive into the crankcase. The percentage change in the brake specific fuel consumption (BSFC) measurement between pre and post sump dosing are shown in the Table below with the data expressed as an average of the test conditions for ease of comparison.

**Table 5**

| | *Test* | *Concentration* | *Average BSFC* |
|---|---|---|---|
| A | NULL | | -0.03% |
| B | CH-5 | 1%v | 0.86% |
| C | CH-5 | 2%v | 1.36% |
| D | CH-5 | 4%v | 1.24% |
| E | CH-2C | 2%v | 0.27% |
| F | CH-6 | 2%v | 0.15% |
| G | Ethomeen T12e | 2%v | 1.19% |
| H | Keracom 3561 | 2%v | 1.36% |
| I | FM10 | 2%v | 1.23% |
| J | Synfluid PAO-5 | 2%v | 0.34% |
| K | Ethomeen T12e | 2%v | 1.36% |
| L | PAO2 (Durasyn 162) | 10%v | 0.48% |
| M | Ethomeen T12e + PAO2 (Durasyn 162) | Ethomeen T12e (2%v) + PAO2 (10%v) | 2.17% |
| N | Ethomeen T12e | 2%v | 1.57% |
| O | Ethomeen 015 | 2%v | 1.24% |
| P | FM10 +Synfluid PAO5 | FM10(2%v) +PAO5 (10%v) | 1.29% |
| Q | FM10 + Priolube 3970 | FM10(2%v) + Priolube 3970(10%v) | 1.31% |
| R | Ethomeen 015 + Synfluid PAO5 | Ethomeen 015 (2%v)+ PAO5 (10%v) | 1.26% |

This example confirms that both friction modifiers and VCA chemistry can cause an increase in % benefit fuel consumption when present in the lubricant. A combination of both friction modifiers and VCA components show an increase in % benefit in fuel consumption over and above an additive increase.

The combined results of Examples 2 and 4 show the benefit of using both friction modifiers and VCA in fuel additive formulations to improve fuel consumption, i.e. to improve fuel economy.

## Claims

1. A liquid fuel composition comprising:
(a) a base fuel suitable for use in an internal combustion engine, wherein the base fuel is a gasoline fuel;
(b) a first fuel additive selected from one or more viscosity control agents having:
(i) a kinematic viscosity at 100°C of 27 mm²/s or less; and
(ii) a NOACK volatility at 250°C of 100 %wt or less; and
(c) a second fuel additive selected from one or more friction modifiers, wherein the one or more friction modifiers is selected from alkoxylated amines;
wherein the first fuel additive is PAO-2, and wherein the liquid fuel composition is a gasoline fuel composition.

2. A liquid fuel composition according to claim 1, wherein the amount of the second fuel additive present in the liquid fuel composition is at least 10 ppmw, and preferably at most 2 wt%, based on the overall weight of the liquid fuel composition.

3. A liquid fuel composition according to any of Claims 1 to 2, wherein the first fuel additive has a kinematic viscosity at 100°C in the range of from 2 mm²/s to 8 mm²/s

4. A liquid fuel composition according to any of Claims 1 to 3, wherein the amount of first fuel additive present in the liquid fuel composition is in the range of from 5 ppmw to 5 %wt, based on weight of the liquid fuel composition.

5. A method of improving the fuel economy performance of an internal combustion engine, said method comprising fuelling the internal combustion engine containing a lubricant with a liquid fuel composition according to any of Claims 1 to 4.

## Patentansprüche

1. Flüssige Kraftstoffzusammensetzung, umfassend:
(a) einen Basiskraftstoff, der zur Verwendung in einem Verbrennungsmotor geeignet ist, wobei der Basiskraftstoff ein Benzinkraftstoff ist;
(b) einen ersten Kraftstoffzusatz, ausgewählt aus einem oder mehreren Viskositätsregulierungsmitteln mit:
(i) einer kinematischen Viskosität bei 100 °C von 27 mm²/s oder weniger; und
(ii) einer NOACK-Volatilität bei 250 °C von 100 Gew.-% oder weniger; und
(c) einem zweiten Kraftstoffadditiv, ausgewählt aus einem oder mehreren Reibungsmodifizierungsmitteln,
wobei das eine oder die mehreren Reibungsmodifizierungsmittel ausgewählt sind aus alkoxylierten Aminen;wobei das erste Kraftstoffadditiv PAO-2 ist, und
wobei die flüssige Kraftstoffzusammensetzung eine Benzin-Kraftstoffzusammensetzung ist.

2. Flüssige Kraftstoffzusammensetzung nach Anspruch 1, wobei die Menge des in der flüssigen Kraftstoffzusammensetzung vorhandenen zweiten Kraftstoffadditivs mindestens 10 ppm und vorzugsweise höchstens 2 Gew.-%, bezogen auf das Gesamtgewicht der flüssigen Kraftstoffzusammen-setzung, beträgt.

3. Flüssige Kraftstoffzusammensetzung nach einem der Ansprüche 1 bis 2, wobei das erste Kraftstoffadditiv eine kinematische Viskosität bei 100 °C im Bereich von 2 bis 8 mm²/s aufweist.

4. Flüssige Kraftstoffzusammensetzung nach einem der Ansprüche 1 bis 3,
wobei die Menge des ersten Kraftstoffadditivs, das in der flüssigen Kraftstoffzusammensetzung vorhanden ist, im Bereich von 5 ppm bis 5 Gew.-% liegt, bezogen auf das Gewicht der flüssigen Kraftstoffzusammensetzung.

5. Verfahren zur Verbesserung der Kraftstoffeinsparleistung eines Verbrennungsmotors, wobei das Verfahren das Betanken des einen Schmierstoff enthaltenden Verbrennungsmotors mit einer flüssigen Kraftstoffzusammensetzung nach einem der Ansprüche 1 bis 4 umfasst.

## Revendications

1. Composition de carburant liquide comprenant :
(a) un carburant de base, convenant pour un usage dans un moteur à combustion interne, le carburant de base étant un carburant de type essence ;
(b) un premier additif pour carburant choisi parmi au moins un agent de régulation de viscosité présentant :
(i) une viscosité cinématique à 100 °C inférieure ou égale à 27 mm²/s ; et
(ii) une volatilité NOACK à 250 °C inférieure ou égale à 100 % en poids ; et
(c) un second additif pour carburant, choisi parmi au moins un agent de modification du frottement, l'au moins un agent de modification du frottement étant choisi parmi les amines alcoxylées ;
le premier additif de carburant étant du PAO-2, et la composition de carburant liquide étant une composition de carburant de type essence.

2. Composition de carburant liquide selon la revendication 1, dans laquelle la quantité du second additif pour carburant présent dans la composition de carburant liquide vaut au moins 10 ppm en poids, et de préférence au moins 2 % en poids, par rapport au poids global de la composition de carburant liquide.

3. Composition de carburant liquide selon l'une quelconque des revendications 1 ou 2, dans laquelle le premier additif pour carburant présente une viscosité cinématique à 100 °C comprise entre 2 mm²/s et 8 mm²/s.

4. Composition de carburant liquide selon l'une quelconque des revendications 1 à 3, dans laquelle la quantité du premier additif pour carburant présent dans la composition de carburant liquide est dans l'intervalle compris entre 5 ppm en poids et 5 % en poids, par rapport au poids de la composition de carburant liquide.

5. Procédé d'amélioration des performances d'économie en carburant d'un moteur à combustion interne, ledit procédé comprenant l'alimentation du moteur à combustion interne contenant un lubrifiant présentant une composition de carburant liquide selon l'une quelconque des revendications 1 à 4.
